

June 19, 1973

E. PELZEL

3,740,214

ZINC ALLOY

Filed Oct. 9, 1970



Erich Pelzel  
Inventor.

By  
Karl G. Ross  
Attorney

1

3,740,214

ZINC ALLOY

Erich Pelze, Puchheim, near Munich, Germany, assignor to Stolberger Zink AG für Bergbau und Hüttenbetrieb, Aachen, Germany

Filed Oct. 9, 1970, Ser. No. 79,533

Claims priority, application Germany, Oct. 25, 1969,  
P 19 53 783.8

Int. Cl. C22c 17/00

U.S. Cl. 75—178 R

5 Claims 10

**ABSTRACT OF THE DISCLOSURE**

A ternary alloy of high-purity zinc, nickel and chromium having high creep resistance and other good mechanical properties for use as bands, strips, sheets, wire or rod which contains Cr and Ni within the area ABCD of the zinc-chromium-nickel composition diagram shown in the drawing wherein A corresponds to 0.05% by weight chromium and 0.05% by weight nickel (balance high-purity zinc), B corresponds to 0.20% by weight chromium and 0.05% by weight nickel (balance high-purity zinc), C corresponding to 0.05% by weight chromium and 0.20% by weight nickel (balance high-purity zinc), and D corresponds to 0.45% by weight to 0.55% by weight chromium and 0.45% by weight to 0.55% by weight nickel (balance high-purity zinc). Up to 1.7% by weight of zinc may be replaced by an equal quantity of copper.

My present invention relates to zinc alloys with improved mechanical properties and, more particularly, to a ternary alloy of zinc, chromium and nickel with improved creep resistance and strength properties.

Numerous zinc alloys have been proposed heretofore for the production of zinc bands, strips, sheet, wire, rods, profiles and bars, for construction and other uses, since elemental zinc, free from alloying ingredients, has poor mechanical properties in many important respects. For example, zinc is prone to creep, i.e. deform under the static load, even at ambient temperatures. Consequently, efforts have been made to increase the tear strength, the ductility and the tensile strength of zinc bodies, while also reducing the tendency to creep. While a review of all of the hitherto disclosed alloys which purport to improve the properties of zinc bodies may only result in confusion, special attention should be given to earlier proposals whereby copper and chromium, copper and titanium, manganese, iron and other alloying metals have been used in varying quantities to modify the physical properties of zinc. For the most part, the prior-art attempts have been unsuccessful in yielding alloys which successfully may be employed in the construction trades, which are sufficiently ductile and creep resistant to be rolled into strips, sheet, bands and the like or to be drawn or rolled into wire and rod, and which yet have the necessary creep resistance. As a matter of fact, it has been found that the crystallography of zinc and zinc alloys is highly complex and that the use of alloying ingredients which themselves appear to improve the creep resistance of zinc, when utilized in combination, does not always provide similar effects or may even destroy some of the improvement already gained. There appears, therefore, to be a significant dependency upon the manner in which the zinc and alloy crystals form in the zinc body, i.e. upon the nature of the eutectoids and the solid solutions formed.

It is, therefore the principal object of the present invention to provide an improved zinc alloy whereby disadvantages of the prior systems are avoided.

It is another object of this invention to provide a zinc alloy particularly suitable for rolling into strip, bands, sheets and the like.

2

It is another object of this invention to provide an improved zinc alloy particularly suitable for drawing into wire and rod.

Still further, it is an object of the invention to provide zinc alloy bodies with high creep resistance and tensile strength.

These objects and others, which will become apparent hereinafter, are attained in accordance with the present invention, with zinc alloys within a well-defined composition range in the ternary composition diagram of high-purity zinc, nickel and chromium. More particularly, we have discovered that there exists in this ternary composition diagram (see the drawing), a region defined by the points A-B which provides the surprising result of low creep and high mechanical strength and ductility.

In the discussion below with respect to the composition, reference is made to "high-purity" zinc. To define this term, it is best to recall that zinc is generally available in a number of grades such as "selected," "brass special," "intermediate," "high-grade" and "special high-grade." The latter two grades are defined for the purposes of the present invention as high-purity zinc. In other words, high-purity zinc is zinc which contains a maximum of 0.07% by weight lead, 0.02% by weight iron and 0.07% by weight cadmium. The sum of the lead, iron and cadmium will not exceed 0.10% by weight. Preferably, however, the high-purity zinc is the "special high-grade" zinc as defined by ASTM specification B 6-49 and contains at most 0.006% by weight lead, 0.005% by weight iron and 0.004% by weight cadmium (total lead, iron and cadmium being at most 0.01% by weight).

The area of the zinc/chromium/nickel ternary composition diagram is the polygon defined by the vertices A, B, C and D wherein:

35 A= 0.05% by weight chromium and  
0.05% by weight nickel,  
balance high purity zinc;

40 B= 0.20% by weight chromium and  
0.05% by weight nickel,  
balance high-purity zinc;

C= 0.05% by weight chromium  
0.20% by weight nickel  
balance high-purity zinc;

D= 0.45% to 0.55% by weight chromium and  
0.45% to 0.55% by weight nickel  
balance high-purity zinc.

Preferably:

55 D= 0.50% by weight chromium and  
0.50% by weight nickel  
balance high-purity zinc.

The points A, B, C and D define lines which constitute phase boundaries and have been observed empirically to define the limits of the operable alloy. The eutectoid of this composition is 0.12% by weight chromium and 0.18% by weight nickel (balance high-purity zinc).

Surprisingly, I have also found that up to 1.7% of the high-purity zinc may be replaced by copper, this amount being the maximum of copper which forms a solid solution in zinc without producing any heterogeneities, lattice or crystalline discontinuities or additional phase boundaries.

In the above-identified eutectic concentration range, the ternary alloy of high-purity zinc, nickel and chromium, in spite of its increasing heterogeneity and increasing solidification interval (as the concentration changes in

the direction of point D) grows more fine-grained, so that the tensile strength increases while the ductility remains. Only when the concentration exceeds that of the point D, i.e. when either 0.5 weight-percent nickel or chromium is exceeded in the composition does this effect cease. While at the outset, it may appear that the range of interest in accordance with the present invention is relatively broad, it should be noted that it constitutes a small fraction only of the range of ternary compositions between 0.05% and 0.5% by weight chromium and between 0.05% and 0.5% by weight nickel.

At the conclusion of primary crystallization, the lattice structure appears to be a pseudoeutectoid in the form of fine crystals and a matrix phase of the ternary eutectic.

The zone of interest, according to the present invention, can be considered to be subdivided into several subzones as will be apparent hereinafter. The point E described below is, of course, the eutectic point. Consequently, the region ABEC, designated  $\alpha$ , solidifies as a fine-grained crystal structure provides the fatigue strength and tensile strength, in major part, of the alloy. The ternary alloy developing in this range has a tensile strength up to 30 kp./mm.<sup>2</sup> and is advantageously rolled into bands, sheets and strips. This ternary alloy has a primary segregation of zinc grains in the eutectoid matrix.

In the phase zone  $\beta$ , defined by the points C, E and D, the primary precipitate is nickel grains which provide a fine-grain structure; the latter, as noted, affords high ductility in spite of the increasing solidification interval and the alloy has been found to be suitable for cold deformation. In the phase zone  $\gamma$ , defined by the points B, E and D, the primary crystals are of chromium with a fine-grain structure and permit, in the presence of copper as noted, tensile strength up to 50 kp./mm.<sup>2</sup> and tensile strength above 50 kp./mm.<sup>2</sup> in copper-containing alloys according to the invention along the phase boundary DE. The ternary alloy in the zone or ridge on either side of the line DE, represented as the region BECD, therefore, has been found to be particularly suitable for the production of wire by drawing.

TABLE

| Example No. | Percent by weight |      |       |           | Tensile strength (kp./mm. <sup>2</sup> ) | Elongation (percent) (to break) | Fatigue strength                         |                     |
|-------------|-------------------|------|-------|-----------|------------------------------------------|---------------------------------|------------------------------------------|---------------------|
|             | Ni                | Cr   | Cu    | Zn        |                                          |                                 | creep resistance (kp./mm. <sup>2</sup> ) | Use                 |
| 1-----      | 0.05              | 0.05 | ----- | Remainder | 18                                       | 70                              | 6                                        | Band, strip, sheet. |
| 2-----      | 0.10              | 0.10 | ----- | do        | 19                                       | 70                              | 6                                        | Do.                 |
| 3-----      | 0.15              | 0.15 | ----- | do        | 20                                       | 80                              | 7                                        | Do.                 |
| 4-----      | 0.25              | 0.15 | ----- | do        | 23                                       | 80                              | 8                                        | Do.                 |
| 5-----      | 0.25              | 0.15 | 1.00  | -----     | 30                                       | 65                              | 9                                        | Do.                 |
| 6-----      | 0.25              | 0.20 | ----- | do        | 25                                       | 60                              | 9                                        | Wire, rod.          |
| 7-----      | 0.35              | 0.30 | ----- | do        | 35                                       | 50                              | 10                                       | Do.                 |
| 8-----      | 0.35              | 0.30 | 1.70  | -----     | 50                                       | 40                              | 10                                       | Do.                 |
| 9-----      | 0.40              | 0.45 | ----- | do        | 40                                       | 15                              | 11                                       | Do.                 |
| 10-----     | 0.50              | 0.50 | ----- | do        | 50                                       | 10                              | 12                                       | Do.                 |

The above examples illustrate the invention, the table giving the composition, tensile strength, elongation to break, fatigue strength or creep resistance and use of ten compositions in accordance with the present invention.

The alloys of Examples 1-5 are cast at 450° C. into blocks with a thickness of 80 mm. After solidification, the blocks are rolled into ductile high-elongability sheets or bands at a temperature of 250° C. in a number of rolling steps to a thickness of 10 mm. (hot-rolling), thereafter the sheets are rolled in several passes to a thickness of 1 mm. (cold-rolling).

In Example 5, 1.00% of the zinc is replaced by copper, thereby increasing the tensile strength to 30 kp./mm.<sup>2</sup> without affecting its elongation to break.

Examples 6-10 were carried out by extruding the alloy from a molten state at 450° C. to round bars of 150 mm. diameter. The bars were then hot-pressed at 250° C. and drawn cold to wire with a diameter of 1.5 mm. In Example 8, 1.7% of the zinc was replaced by copper and the tensile strength of the wire was thereby increased to 50 kp./mm.<sup>2</sup>.

The products according to the present invention were of increased hardness and tensile strength and high elongability.

I claim:

1. A ternary zinc/nickel/chromium alloy consisting essentially of 0 to 1.7% by weight copper, and nickel and chromium in amounts within the area ABCD of the drawing, balance high-purity zinc, wherein

A= 0.05% by weight chromium and  
0.05% by weight nickel;

B= 0.20% by weight chromium and  
0.05% by weight nickel;

C= 0.05% by weight chromium and  
0.20% by weight nickel; and

D= 0.45% to 0.55% by weight chromium and  
0.45% to 0.55% by weight nickel.

2. The alloy defined in claim 1 wherein

D= 0.50% by weight chromium and  
0.50% by weight nickel.

3. The alloy defined in claim 1 having a ternary eutectic point of  
0.12% by weight chromium and  
0.18% by weight nickel.

4. A sheet zinc alloy rolled from the composition defined in claim 1 and within the area ABCE of the drawing.

5. Wire drawn from the composition defined in claim 1 and within the area ADCE of the drawing.

## References Cited

## UNITED STATES PATENTS

- 3,527,601 9/1970 Foerster ----- 75-178 R  
2,011,987 8/1935 Tainton et al. ----- 75-178 R  
1,506,772 9/1924 Pack ----- 75-178 R

## FOREIGN PATENTS

- 1,319,535 1/1963 France ----- 75-178 R

L. DEWAYNE RUTLEDGE, Primary Examiner

E. L. WEISE, Assistant Examiner

U.S. CL. X.R.

75-178 C

UNITED STATES PATENT OFFICE  
CERTIFICATE OF CORRECTION

Patent No. 3,740,214 Dated June 19, 1973

Inventor(s) Erich Pelzel

It is certified that error appears in the above-identified patent and that said Letters Patent are hereby corrected as shown below:

Column 1, line 3, "Erich Pelze" should read

-- Erich Pelzel --.

Signed and sealed this 26th day of February 1974.

(SEAL)

Attest:

EDWARD M.FLETCHER, JR.  
Attesting Officer

C. MARSHALL DANN  
Commissioner of Patents